

[54] SILVER HALIDE EMULSIONS  
CONTAINING TWO-EQUIVALENT  
BENZOYLACETANILIDE PHOTOGRAPHIC  
COUPLERS

[75] Inventor: **Andrea Quaglia, Albisola Mare, Italy**

[73] Assignee: **Minnesota Mining and Manufacturing Company, St. Paul, Minn.**

[22] Filed: **Dec. 26, 1972**

[21] Appl. No.: **318,561**

[30] **Foreign Application Priority Data**

Dec. 28, 1971 Italy ..... 55062/71

[52] U.S. Cl. .... **96/100; 96/56; 260/562 B**

[51] Int. Cl. .... **G03c 1/40**

[58] **Field of Search** ..... 96/100, 55

[56]

**References Cited**

**UNITED STATES PATENTS**

|           |         |                   |        |
|-----------|---------|-------------------|--------|
| 3,056,675 | 10/1962 | Hoffstadt .....   | 96/100 |
| 3,369,895 | 2/1968  | Loria et al. .... | 96/100 |
| 3,664,841 | 5/1972  | Iwama et al. .... | 96/100 |
| 3,669,671 | 6/1972  | Iwama et al. .... | 96/100 |

*Primary Examiner*—J. Travis Brown

*Attorney, Agent, or Firm*—Alexander, Sell, Steldt & DeLaHunt

[57] **ABSTRACT**

Two-equivalent benzoylacetanilide photographic couplers containing ballasting groups attached to an aromatic ring thereof characterized by a halogen atom in ortho position in the benzoyl residue and a halogen atom as a substituent in the reactive methylene which are substantially free of fog and produce yellow dyes substantially without orange coloration upon color development.

**3 Claims, No Drawings**

**SILVER HALIDE EMULSIONS CONTAINING  
TWO-EQUIVALENT BENZOYLACETANILIDE  
PHOTOGRAPHIC COUPLERS**

The present invention relates to two-equivalent benzoylacetanilide couplers for color photography and to colored photographic elements containing them.

More specifically the present invention relates to two-equivalent benzoylacetanilide couplers which give rise to yellow dyes upon color development with p-phenylene diamine type developers.

The present invention further relates to photographic emulsions containing such couplers, to photographic elements including such emulsions and to photographic elements containing the dyes derived from such couplers upon color development.

Colored photographic elements normally include at least three emulsion layers which are sensitive to the blue, to the green and to the red region and contain, respectively, a yellow, a magenta and a cyan coupler.

It is recognized in the art that couplers used in photographic elements should not be excessively reactive. This will prevent undesired color formations.

It is also known that couplers must give rise upon color development to dyes having a given desired absorption curve to obtain images with "balanced colors." It may be useful, for instance, to obtain yellow dyes substantially without orange colorations, i.e., with a low absorption in the green region.

Benzoylacetanilide type couplers are capable of reacting with the oxidation product of p-phenylene diamine type developers to form yellow images in light exposed silver halide photographic elements.

Upon color development with p-phenylene diamine type developers, a molecule of such couplers normally give rise to a molecule of a dye by the reduction of four silver ions struck by the light. If however one of the hydrogens of the reactive methylene in the coupler is substituted with a suitable substituent, a molecule of a dye can be obtained by the reduction of only two silver ions.

The couplers which exhibit such characteristics are commonly called two-equivalent couplers: the meaning of this expression is clear. Obviously they are very useful in color photographic industry because they allow a lower consumption of silver in color photographic emulsions which employ incorporated couplers.

Benzoylacetanilide couplers include a benzoyl residue (phenyl-CO) and an aniline residue (NH-phenyl) joined by a carboxymethylene bridge (CH<sub>2</sub>-CO). This methylene group is called "reactive methylene" because the coupling reaction occurs on it.

Two-equivalent benzoylacetanilide couplers are described for instance in the French Pat. No. 991,453; in U.S. Pat. Nos. 2,407,210; 2,728,658; 3,408,194; 3,447,928 and in the British Pat. No. 1,092,506.

Such two-equivalent benzoylacetanilide couplers have some drawbacks which make their practical employment in colored photographic elements difficult and sometimes impossible. These difficulties drive from their excessive reactivity which enables them to react with the developer even in absence of exposed silver halide, thus giving rise to undesired coloration commonly called "fog." Furthermore, some two-equivalent benzoylacetanilide couplers known in the art are much more expensive than four-equivalent couplers from

which they derive. This higher cost is due to synthesis difficulties.

The present invention mainly refers to low-cost two-equivalent benzoylacetanilide couplers which are substantially free of fog effects in photographic silver halide emulsions.

More specifically it relates to low-cost two-equivalent benzoylacetanilide couplers substantially free of fog which give rise, upon color development, to yellow dyes substantially without orange coloration.

According to the present invention, it was found that low-cost couplers substantially free of fog can be obtained by the combination of a halogen substituent (Y) in ortho position in the benzoyl and a halogen substituent (X) in the reactive methylene.

It was further found that a fluorine atom as a substituent in ortho position in the benzoyl and a halogen atom as a substituent in the reactive methylene yield low-cost benzoylacetanilide couplers, substantially free of fog, which give rise to yellow dyes substantially without orange coloration upon color development with p-phenylene diamines.

The halogen substituent (X) produces low-cost two-equivalent couplers, and the halogen substituent (Y), combined with it, yields two-equivalent couplers substantially free of fog.

The halogen substituent in ortho position in the benzoyl is an essential substituent for the purposes of the present invention. It enables one to obtain, free of fog, two-equivalent benzoylacetanilide couplers of the type having a hydrogen of the reactive methylene substituted with a halogen.

Other substituents can obviously be introduced into the benzoyl and aniline residues to provide the couplers or the dyes deriving therefrom upon color development with desired characteristics. For example, these characteristics may relate to the solubility of the couplers, to their non-diffusing properties, to the stability of the dyes deriving therefrom and to their absorption characteristics. Such substituents however are thought to be of secondary importance for the main purpose of the present invention. The man ordinarily skilled in the art can select them readily, so that the advantages of the present invention can be achieved and the requirements of particular usages satisfied everytime.

Substituents which can be usefully introduced into the molecule of the couplers of the present invention are for instance alkyl groups (having for instance from 1 to 18 carbon atoms), halogen (for instance Cl, Br, F), alkoxy groups (having for instance from 1 to 18 carbon atoms), dialkylamino groups (having from 2 to 19 carbon atoms), arylaminosulphonyl groups (for instance phenylaminosulphonyl, alkylphenylaminosulphonyl, o- and p-alkylphenylaminosulphonyl, o- and p-alkoxyphenylaminosulphonyl, wherein the alkyl or alkoxy group has from 1 to 18 carbon atoms), aryloxacylaminogroup (for instance phenoxyacylaminogroup, phenoxyacetylaminogroup, alkylphenoxyacetylaminogroup, 2,4-dialkyl-phenoxyacetylaminogroup, 2,4-dialkylphenylacetylaminogroup, wherein the alkyl group or the alkyl groups have altogether from 1 to 18 carbon atoms, acyl group having from 1 to 18 carbon atoms, arylsulphonamido (for instance phenylsulphonamido, alkylphenylsulphonamido, alkoxyphenylsulphonamido, o- and p-alkylphenylsulphonamido, o- and p-alkoxyphenylsulphonamido, wherein the alkyl or alkoxy group has from 1 to 18 carbon atoms) and every other

substituent known to the man ordinarily skilled in the art. The applicant has observed that the best substituent combination to obtain, within the scope of the present invention, two-equivalent couplers free of fog which give rise to yellow dyes substantially without orange coloration upon color development with p-phenylene diamine type developers is the combination of a fluorine atom in the ortho position in the benzoyl, a halogen in the reactive methylene and an electron donor of the alkyl, alkoxy group, dialkylamino type and their equivalents in ortho position in the aniline residue. Very stable couplers within the present invention can be further obtained if in combination with the halogen, particularly fluorine atom in ortho position in the benzoyl, the halogen in the reactive methylene and the electron donor of the alkyl, alkoxy group and dialkylamino type in 2 (ortho) position in the aniline residue, an arylsulphonamido or arylaminosulphoxy group in 5-position in the aniline residue (for instance phenylaminosulphoxy, alkylphenylaminosulphoxy, alkoxyaminosulphoxy, o- and p-alkylphenylaminosulphoxy, o- and p-alkoxyphenylaminosulphoxy, phenylsulphonamido, alkylphenylsulphonamido, alkoxyphenylsulphonamido, o- and p-alkylphenylsulphonamido, o- and p-alkoxyphenylsulphonamido, wherein the alkyl or alkoxy group has from 1 to 18 carbon atoms) is used.

It is desirable for a correct employment of the couplers of the present invention in silver halide photographic emulsions to provide them with ballasting groups which prevent them from wandering through the emulsion layers that compose the silver halide photographic elements. In view of this, the coupler is intended to mean a "non-diffusing coupler," i.e., a coupler carrying at least a ballasting group capable of imparting non-diffusing properties to the said coupler. The ballasting groups or anti-diffusing chains, as they are often called, (generally comprising high-molecular weight alkyl groups, e.g., having from 10 to 18 carbon atoms) can be introduced as substituents either into the benzoyl residue or into the aniline residue of the couplers of the present invention, because it does not appear that they substantially affect the coupler characteristics necessary for the purposes of the present invention. On account of preparation ease, and therefore of cost, the ballasting group is preferably introduced into the aniline residue, preferably into the phenyl ring in ortho (2) and/or in meta (5) position to the carbon atom carrying the amino group (briefly: in ortho and/or in meta position in the aniline residue).

In the case where the couplers of the present invention must be incorporated into photographic emulsions in aqueous solution, they must be made water-soluble by means of the  $\text{SO}_3\text{H}$  and  $\text{COOH}$  type. In the case where they must be incorporated into the emulsion by the solvent dispersion technique, the couplers must be soluble in substantially water-immiscible organic solvents (see: C. E. Kenneth Mees and T. H. James, *The Theory of Photographic Process*, third edition, page 303).

Such techniques, which are now preferred, are described for instance in U.S. Pat. Nos. 2,322,027; 2,801,170; 2,801,171; 2,870,012 and 2,991,177. Briefly the solvent dispersion technique involves first 10 dissolving a coupler in a substantially water-immiscible organic solvent and then dispersing the so-prepared solution as extremely fine droplets in a hydrophilic colloidal binder. Gelatin is the preferred hydrophilic colloidal binder but other polymeric colloidal binder materials known to the art can also be used. Obviously, when the couplers are incorporated into the emulsion by the solvent dispersion technique, the dyes deriving therefrom upon color development are also contained dispersed in the emulsion dissolved in the substantially water-immiscible organic solvent.

Briefly, the present invention refers, in its most general aspects, to non-diffusing benzoylacetanilide couplers including a halogen atom in the reactive methylene and in ortho position in the benzoyl residue as expressed by the following formula:



wherein: B is a benzoyl residue bearing a halogen substituent in the phenyl in the ortho position to the carbon atom carrying the carbonyl; X represents a halogen atom and A is an aniline residue.

In its more particular aspect, the present invention refers to non-diffusing benzoylacetanilide couplers containing a halogen substituent in the reactive methylene and a fluorine atom in ortho position in the benzoyl. More particularly, the present invention relates to non-diffusing couplers of the benzoylacetanilide type including a halogen atom, and in particular a fluorine atom, in ortho position in the benzoyl, a halogen atom in the reactive methylene and an electron donor of the alkyl group, alkoxy group, dialkylamino group type in ortho position in the aniline residue. More particularly, the present invention refers to non-diffusing couplers of the benzoylacetanilide type including a halogen atom, and in particular a fluorine atom, in ortho position in the benzoyl residue, a halogen atom in the reactive methylene, an electron donor of the alkyl group, alkoxy group, dialkylamino group type in 2-position in the aniline residue and a group of the arylsulphonamido or arylaminosulphoxy type in 5-position in the same aniline residue.

The present invention also relates to silver halide photographic emulsions containing such couplers preferably introduced by the solvent dispersion technique and to photographic elements comprising such emulsions. The present invention further relates to exposed and developed silver halide photographic elements containing dyes derived from the said couplers upon coupling reaction with p-phenylene diamine type compounds.

Useful couplers within the scope of the present invention are for instance the following:



- 5
- 2) 
- 3) 
- 4) 
- 5) 
- 6) 
- 7) 
- 8) 
- 9) 
- 10) 
- 11) 
- 12) 



Prior art couplers useful for a comparison with the couplers according to the present invention are for example the following.

51.7 g. (0.3 moles) of 3-nitro-4-chloro-aniline, 29.5 g. (0.36 moles) of sodium acetate anhydrous and 450 ml. of glacial acetic acid were mixed in a multi-neck



The following examples further illustrate the practice of the present invention:

#### EXAMPLE 1

$\alpha$ -(2-chlorobenzoyl)- $\alpha$ -chloro-5-[ $\alpha$ -(2-4-ditert-  
amylphenoxy)-acetamido]-2-chloroacetonitrile  
Intermediate 1: 3-nitro-4-chloro- $\alpha$ -(2-4-ditertamyl-  
phenoxy)-acetanilide

flask of 1 liter provided with a stirrer and a reflux-condenser. The mixture was stirred till a complete solution was reached and 93.2 g. (0.3 moles of 2-4-ditertamyl-phenoxy-acetyl-chloride) were added thereto. The solution was stirred for 1 hour at room temperature and further at 70°C for half an hour. The hot solution was poured into icy water and the precipitate filtered, washed, dried and crystallized from etha-

nol, thus obtaining 112.4 g. of a white product melting at 154-155°C.

| Analysis: |       | Found | Calculated |
|-----------|-------|-------|------------|
| N%        | 6.26  | 6.24  |            |
| C%        | 64.51 | 64.48 |            |
| H%        | 7.05  | 6.99  |            |

**Intermediate 2: 3-amino-4-chloro- $\alpha$ -(2-4-ditertamyl-phenoxy)-acetanilide**

44.6 g. (0.1 moles) of the intermediate 1 were put into a 500 ml. autoclave with 250 ml. of ethanol and Ni Raney in catalytic quantities. The mixture was held under stirring for 10 h at a H<sub>2</sub> pressure of 40 atm. and at a temperature of 50°C. The Ni was removed from the solution by filtration, the solution was then dried and the residue crystallized from ligroin, thus obtaining 31.8 g. of a white product melting at 110°-112°C.

Analysis: -NH<sub>2</sub>% = 98.7

**Intermediate 3:  $\alpha$ -(2-chlorobenzoyl)-5-[ $\alpha$ -(2-4-ditertamylphenoxy)-acetamide]-2-chloro-acetanilide**

41.7 g. (0.1 moles) of the intermediate 2 and 200 ml. of xylene were mixed into a multi-neck flask provided with a stirrer and a Liebig condenser. To the solution brought to boil, 10 ml. of a solvent distilled and 24.9 g. (0.11 moles) ethyl o-chlorobenzoyl acetate, prepared according to the method described in J.A.C.S. 37, 1259, were added thereto. The solution was boiled gently for 3 h, thus obtaining 40 ml. of distillate. The precipitate thus formed was filtered, washed with dried methanol and recrystallized from methanol, thus obtaining 33.5 g. of a white product melting at 108°-110°C.

| Analysis:                                  |       | Found | Calculated |
|--------------------------------------------|-------|-------|------------|
| Cl%                                        | 11.81 | 11.87 |            |
| Titration from >CH <sub>2</sub> % = 99.88. |       |       |            |

**Preparation of the coupler**

20.8 g. (0.0348 moles) of  $\alpha$ -(2-chlorobenzoyl)-5-[ $\alpha$ -(2-4-ditertamylphenoxy)-acetamide]-2-chloroacetanilide and 100 ml. of anhydrous chloroform were mixed into a 250 ml. multi-neck flask provided with a stirrer and a refluxe-condenser. The solution was cooled at some 5°C and 4.4 g. (0.034 moles) of pure sulphonylchloride all at once added thereto. The mixture was held under stirring for 3 h at room temperature, afterwards the solvent was distilled under vacuum and the molten residue dissolved in boiling methanol. The precipitation of a white-rosy product was obtained by cooling the solution. The precipitate was recrystallized from methanol, thus obtaining 17.5 g. of a white product melting at 95°-98°C.

| Analysis:                    |      | Found | Calculated |
|------------------------------|------|-------|------------|
| Cl%                          | 16.7 | 16.83 |            |
| Titration from →CH% = 99.95. |      |       |            |

**EXAMPLE 2**

**$\alpha$ -(2-chlorobenzoyl)- $\alpha$ -chloro-2-methoxy-5-[ $\alpha$ -(2-4-ditertamylphenoxy)-acetamide]-acetanilide**

**Intermediate 4:  $\alpha$ -(2-chlorobenzoyl)-2-methoxy-5-nitro-acetanilide**

50.5 g. (0.3 moles) of 2-methoxy-5-nitro-aniline and 200 ml. of xylene were mixed into a 500 ml. multi-neck flask provided with a stirrer and a Liebig condenser. The mixture was brought to boil and when some 10 ml. of solvent were distilled, 81.6 g. (0.36 moles) of ethyl 2-chlorobenzoylacetate were added thereto. The solution was boiled gently for 4 h., thus obtaining 35 ml. of distillate and afterwards cooled at room temperature and then at 3°-5°C for 2 h.

10 The precipitate thus formed was filtered, washed first with xylene and then with petroleum ether, dried and finally recrystallized from acetone, thus obtaining 85 g. of a crystalline straw-colored product melting at 132°-134°C.

| Analysis:                                  |       | Found | Calculated |
|--------------------------------------------|-------|-------|------------|
| Cl%                                        | 10.11 | 10.17 |            |
| Titration from >CH <sub>2</sub> % = 99.65. |       |       |            |

**Intermediate 5:  $\alpha$ -(2-chlorobenzoyl)-2-methoxy-5-amino-acetanilide**

25 A 250 ml. methylcellosolve and Ni Raney (in catalytic quantities) solution of 34.8 g. (0.1 moles) of the intermediate 4 was poured into a 500 ml. autoclave. The mixture was stirred for 18 h at room temperature at a H<sub>2</sub> pressure of 35 atm.

30 The Ni was then removed by filtration and the solvent distilled under vacuum. The oily residue was dissolved in boiling methanol. By cooling the solution, a white crystalline precipitate was obtained. The precipitate was then filtered washed and dried, thus obtaining 35 25.6 g. of a product melting at 124°-126°C.

| Analysis:                                |       | Found | Calculated |
|------------------------------------------|-------|-------|------------|
| Cl%                                      | 11.14 | 11.12 |            |
| Titration from NH <sub>2</sub> % = 99.2. |       |       |            |

**Intermediate 6:  $\alpha$ -(2-chlorobenzoyl)-2-methoxy-5-[ $\alpha$ -(2-4-ditertamyl-phenoxy)-acetamide]-acetanilide**

9.2 g. (0.13 moles) of sodium acetate anhydrous were dissolved into 400 ml. of glacial acetic acid in a 1 l. multi-neck flask provided with a stirrer and refluxe condenser.

50 30 g. (0.094 moles) of the intermediate 5 and further 29.2 g. (0.094 moles) of 2-4-ditert-amyl-phenoxy-acetylchloride were then added to the solution. It was then stirred for 1 h at room temperature and 1/2 h at 60°-70°C, the mixture was then poured into icy water under stirring. The precipitate thus formed was filtered, washed with water, dried and recrystallized from ethanol, thus obtaining 40.6 g. of a white product melting at 131°-133°C.

| Analysis:                                 |      | Found | Calculated |
|-------------------------------------------|------|-------|------------|
| Cl%                                       | 5.91 | 5.98  |            |
| Titration from >CH <sub>2</sub> % = 98.6. |      |       |            |

**Coupler 2**

65 This coupler was prepared in the manner described in Example 1.

26.1 g. of a white product, recrystallized from ethanol, were obtained from 29.7 g. (0.05 moles) of the intermediate 6 and 6.8 g. (0.05 moles) of sulphonyl chloride. M. P. 96°-98°C.

| Analysis:                  | Cl% | Found | Calculated |
|----------------------------|-----|-------|------------|
| Titration from CH% = 98.2. |     | 11.27 | 11.29      |

### EXAMPLE 3

$\alpha$ -(2-bromobenzoyl)- $\alpha$ -chloro-5-[ $\alpha$ -(2-4-ditertamylphenoxy)-acetamide]-2-chloroacetanilide

Intermediate 7: ethyl 2-bromobenzoylacetate

This compound was prepared as was ethyl 2-chlorobenzoylacetate according to the method described in J.A.C.S. 37, 1259.

The product, thus obtained, is an oily straw-colored liquid boiling at 155°-158°C/2 mm Hg.

Intermediate 8:  $\alpha$ -(2-bromobenzoyl)-5-[ $\alpha$ -(2-4-ditertamylphenoxy)-acetamide]-2-chloro-acetanilide

This product was prepared in the same manner as intermediate 3.

33.4 g. of a white product, recrystallized from ethanol, were obtained from 61 g. (0.143 moles) of intermediate 2 and 43.3 g. (0.16 moles) of intermediate 7.

| Analysis: | Found | Calculated |
|-----------|-------|------------|
| C%        | 61.84 | 61.73      |
| H%        | 6.04  | 5.97       |
| N%        | 4.44  | 4.36       |

### Coupler 3

This coupler was obtained in the same manner as coupler 1.

23 g. of the product, recrystallized from heptane, were obtained from 25.7 g. (0.04 moles) of intermediate 8, dissolved in 100 ml. of chloroform and 5.4 g. (0.04 moles) of sulphonyl chloride. M. P. 106°-108°C.

| Analysis: | Found | Calculated |
|-----------|-------|------------|
| Cl%       | 10.41 | 10.48      |
| Br%       | 11.79 | 11.81      |

Titration from  $\rightarrow$ CH% = 99.0.

### EXAMPLE 4

$\alpha$ -(2-fluorobenzoyl)- $\alpha$ -chloro-5-[ $\alpha$ -(2-4-ditertamylphenoxy)-acetamide]-2-chloroacetanilide

Intermediate 9: ethyl 2-fluorobenzoylacetate

This product was obtained in the same manner as the corresponding chloro-derivative according to the method described in J.A.C.S. 37, 1259. It is a colorless oil boiling at 104°-106°C 1.5 mm. Hg.

Intermediate 10:  $\alpha$ -(2-fluorobenzoyl)-5-[ $\alpha$ -(2-4-ditertamylphenoxy)-acetamide]-2-chloroacetanilide

This product was prepared in the same manner as intermediate 3.

35.6 g. of a white product, recrystallized from methanol, were obtained from 63 g. (0.151 moles) of the intermediate 2, 375 ml. of xylene and 34 g. (0.162 moles) of ethyl 2-fluorobenzoylacetate. M. P. 137°-139°C.

| Analysis: | Found | Calculated |
|-----------|-------|------------|
| C%        | 68.36 | 68.18      |
| H%        | 6.59  | 6.59       |
| N%        | 4.71  | 4.82       |
| Cl%       | 6.13  | 6.10       |

5 Titration from  $\text{--CH}_2$  = 99%

### Coupler 4

This coupler was prepared in the same manner as coupler 1.

23.2 g. of a white product, recrystallized from methanol, were obtained from 23.2 g. (0.04 moles) of intermediate 10, dissolved in 100 ml. of chloroform anhydrous and 5.4 g. (0.04 moles) of sulphonyl chloride.

| Analysis: | Found | Calculated |
|-----------|-------|------------|
| Cl%       | 11.37 | 11.54      |

10 Titration from  $\rightarrow$ CH% = 99.19.

### EXAMPLE 5

$\alpha$ -(2-chlorobenzoyl)- $\alpha$ -chloro-2-cetoxyacetanilide

Intermediate 11; 2-cetoxy-nitrobenzene

8.3 g. (0.36 moles) of metallic sodium were added in small portions into a 1 l. multi-neck flask provided with a stirrer, a thermometer, a dropping funnel and refluxe-condenser and containing 325 ml. of cellosolve. The mixture was stirred till a complete solution was reached and cooled at 20°C. 50 g. (0.36 moles) of o-nitrophenol were then added thereto in small portions. After 30 minutes of stirring, 110.5 g. (0.36 moles) of cetyl bromide were added thereto dropwise, the mixture was boiled for 5 h. and then poured into icy water. The precipitate, thus obtained, was filtered, washed till  $\text{Br}^{116}$  was removed completely, dried and recrystallized from ethanol, thus obtaining 152 g. of a product melting at 33°-35°C.

| Analysis: | Found | Calculated |
|-----------|-------|------------|
| C%        | 72.70 | 72.69      |
| H%        | 10.25 | 10.26      |
| N%        | 3.92  | 3.86       |

50 Intermediate 12: 2-cetoxy-aniline

By reduction with hydrogen in an autoclave and using Ni Raney as a catalyst, 88.6 g. of a white product were obtained from 109 g. (0.3 moles) of intermediate 11 dissolved in 1 liter of ethanol. M.P. 50°-52°C.

55 Analysis: Titration from  $\text{NH}_2$  = 99.2 percent  
Intermediate 13:  $\alpha$ -(2-chlorobenzoyl)-2-cetoxyacetanilide

This product was prepared in the same manner as intermediate 3.

60 38.8 g. of a white product, recrystallized from ethanol, were obtained from 24.8 (0.1 moles) of ethyl 2-chlorobenzoylacetate and 33.3 g. (0.1 moles) of o-cetoxyaniline (intermediate 12). M.P. 65°-66°C.

| Analysis: | Found | Calculated |
|-----------|-------|------------|
| Cl%       | 6.88  | 6.90       |

65 Titration from  $\text{--CH}_2$  = 99.35%.

## Coupler 5

This coupler was prepared in the same manner as coupler 1.

27 g. of a crystalline white product, recrystallized from isopropylic alcohol, were obtained from 50.8 g. (0.06 moles) of intermediate 13 and 8.1 g. (0.06 moles) of sulphuryl chloride. M.P. 58°-60°C.

| Analysis:                 | Cl% | Found | Calculated |
|---------------------------|-----|-------|------------|
| Titration from CH% = 98.6 |     | 12.95 | 12.96      |

## EXAMPLE 6

 $\alpha$ -(2-fluorobenzoyl)- $\alpha$ -chloro-2-cetoxyacetanilide

Intermediate 14:  $\alpha$ -(2-fluorobenzoyl)-2-cetoxyacetanilide

This product was prepared in the same manner as intermediate 3.

32.3 g. of a product, crystallized first from ethanol and afterwards from ligroin, were obtained from 27.6 g. (0.0828 moles) of 2-cetoxyaniline (intermediate 12) dissolved in 200 ml. of xylene and 17.4 g. (0.0828 moles) of ethyl 2-fluorobenzoylacetate (intermediate 9). M.P. 70°-72°C.

Analysis: Titration from  $\text{CH}_2$  = 98.2 percent.

## Coupler 6

This coupler was prepared in the same manner as coupler 1.

29 g. of a white product, crystallized from isopropylic alcohol, were obtained from 30.7 g. (0.0616 moles) of intermediate 14, dissolved in 150 ml. of dry chloroform and 8.3 g. (0.0616 moles) of sulphuryl chloride. M.P. 80°-82°C.

| Analysis:                            | Cl% | Found | Calculated |
|--------------------------------------|-----|-------|------------|
| Titration from $\text{CH}_2$ = 98.6% |     | 6.64  | 6.66       |

## EXAMPLE 7

 $\alpha$ -(2-chlorobenzoyl)- $\alpha$ -chloro-2-(N-methyl-N-octadecylamino)-5-sulphanilide-acetanilide

Intermediate 15: 3-nitro-4-chlorobenzensulphanilide

128 g. (0.5 moles) of 3-nitro-4-chlorobenzensulphochloride, 1,000 ml. of acetonitrile anhydrous and 93.2 g. (1 mol) of aniline were mixed into a multi-neck flask provided with stirrer and refluxe-condenser. The solution was boiled for 2 h. and poured into a 5 percent icy solution of HCl. The oily product, which deposited after some hours, coagulated into a solid mass which was filtered, washed till it became neutral, dried and crystallized from carbon tetrachloride, thus obtaining 129.1 g. of a yellow crystalline product, melting at 85°-87°C.

| Analysis: | Found | Calculated |
|-----------|-------|------------|
| C%        | 46.09 | 46.08      |
| H%        | 2.78  | 2.90       |
| N%        | 9.12  | 8.95       |
| Cl%       | 11.26 | 11.33      |

Titration from  $-\text{NO}_2$  = 99.15%.

Intermediate 16: 3-nitro-4-(N-methyl-N-octadecylamino)-benzensulphanilide

31.2 (0.1 moles) of 3-nitro-4-chlorobenzensulphochloride (intermediate 15) and 60 ml. of n-propanol were mixed into a 500 ml. multi-neck flask provided with a stirrer and refluxe condenser. The mixture was heated till a complete solution was reached and an n-propanol (60 ml.) hot solution of 56.7 g. (0.2 moles) of methylocatadecylamine was added thereto. The solution was refluxed for 15 h., poured into icy water and the pH value arranged at 3-4 with HCl. The orange-colored solid, which separated, was filtered, washed and extracted with ethyl ether.

The ethereal solution was dried and evaporated and the yellow residue, thus obtained, was crystallized first from ethanol and then from heptane, thus obtaining 28 g. of a crystalline product under the form of gleaming yellow scales. M.P. 61°-63°C.

| Analysis: | Found | Calculated |
|-----------|-------|------------|
| C%        | 66.99 | 66.51      |
| H%        | 8.93  | 8.82       |
| N%        | 7.71  | 7.50       |

Intermediate 17: 3-amino-4-(N-methyl-N-octadecylamino)-benzensulphanilide

This product was obtained by catalytic reduction in an autoclave of the corresponding nitro-derivative (intermediate 16) using Ni Raney as a catalyst, thus obtaining 18 g. of a product crystallized from ethanol. M.P. 62°-65°C.

Analysis: Titration from  $-\text{NH}_2$  = 97.5 percent.

Intermediate 18:  $\alpha$ -(2-chlorobenzoyl)-2-(N-methyl-N-octadecylamino)-5-sulphanilide-acetanilide

After crystallization from methanol, 26.4 g. of a white product were obtained from 45.7 g. (0.0864 moles) of intermediate 17 and 19.6 g. (0.0864 moles) of ethyl 2-chlorobenzoylacetate, kept at a temperature of 145°C for 2 h. in a rotating flask under vacuum. M.P. 54°-56°C.

| Analysis:                                                | Found | Calculated |
|----------------------------------------------------------|-------|------------|
| Cl%                                                      | 4.93  | 4.99       |
| Acidimetric titration from $-\text{CH}_2$ = 97.2%        |       |            |
| Acidimetric titration from $-\text{SO}_2\text{NH}$ = 97% |       |            |

## Coupler 7

This coupler was prepared in the same manner as coupler 1.

21 g. of the product were obtained from 25 g. (0.035 moles) of intermediate 18 and 4.7 g. (0.035 moles) of sulphuryl chloride. M.P. 43°-47°C.

| Analysis: | Found | Calculated |
|-----------|-------|------------|
| Cl%       | 9.72  | 9.52       |

## EXAMPLE 8

 $\alpha$ -(2-chlorobenzoyl)- $\alpha$ -chloro-5-[(4-dodecyl-phenyl-amino)-sulphoxy]-2-methoxy-acetanilide

Intermediate 19: 3-nitro-4-methoxy-benzensulpho-4-dodecylanilide

13.1 g. (0.05 moles) of parado'cylaniline, 70 ml. of tetrahydrofuran and 7.6 g. (0.075 moles) of triethylamine were mixed into a 250 ml. multi-neck flask provided with a stirrer, a refluxe-condenser and a dropping

funnel. The solution was cooled at 5°C and a tetrahydrofuran (30 ml.) solution of 12.5 g. (0.05 moles) of 3-nitro-4-methoxybenzensulphochloride was added in 15 minutes thereto dropwise under stirring and maintaining a temperature ranging from 5° to 10°C.

After such an addition, the suspension was stirred at 5°-10°C for still another hour and then at 50°C for one-half h. After having been cooled in icy water, the mixture was filtered to remove the white precipitate which deposited and the filtrate was dried by evaporation under vacuum. The yellow oily residue was resolved in 200 ml. of ethyl ether and the solution shaken into a separatory funnel with 200 ml. of current water containing 1.5 ml. of concentrated HCl and washed with water till it became neutral. The water was removed with sodium sulphate anhydrous and the remaining solution dried. The residue was then resolved in 500 ml. of petroleum ether. A white solid was immediately formed which was filtered and recrystallized from ligroin, thus obtaining 15.6 g. of a product melting at 82°-84°C.

Analysis: Titration from  $-\text{NO}_2$  = 99.71 percent.

Intermediate 20: 3-amino-4-methoxy-benzensulpho-4-dodecylanilide

19 g. (0.04 moles) of intermediate 19, 120 ml. of 90 percent acetic acid and 60 ml. of ethanol were mixed into a 500 ml. multi-neck flask provided with a stirrer and refluxe-condenser. The mixture was brought to boil and 22.4 g. (0.4 moles) of pulverized iron were added thereto cautiously in small portions and controlling the addition speed so that the mixture could be kept under light spontaneous boiling. After the additions, the mixture was boiled for another one-half h., filtered when it was boiling and the filtrate was poured, when hot, into icy water. The granulose product which deposited, was isolated, dried and crystallized from methanol, thus obtaining 12.3 g. of a pink-colored product melting at 121°-123°C.

Analysis: Titration from  $-\text{NH}_2$  = 100.0 percent.

Intermediate 21:  $\alpha$ -(2-chlorobenzoyl)-5-[(4-dodecylamino)sulpho]-2-methoxyacetanilide

This product was obtained in the same manner as intermediate 18.

40.1 g. (0.09 moles) of intermediate 20 and 21.4 g. (0.04 moles) of ethyl 2-chlorobenzoylacetate were mixed and heated up to 145°C in a rotating flask under vacuum for 2 h. The amber-colored molten reaction mixture was crystallized from cyclohexane, thus obtaining 28.6 g. of a product melting at 60°-65°C.

Analysis: Cl% Found 5.68 Calculated 5.65

#### Coupler 8

This coupler was prepared in the same manner as coupler 1.

31.4 g. (0.05 moles) of intermediate 20 dissolved in 150 ml. of chloroform anhydrous were brought to react with 6.7 g. (0.05 moles) of sulphurylchloride, thus obtaining 24 g. of a product crystallized from heptane. M.P. 85°-88°C.

5

#### EXAMPLE 9

$\alpha$ -(2-chlorobenzoyl)- $\alpha$ -chloro-2-methyl-5-laurooyl-acetanilide

#### Intermediate 22: 3-nitro-4-methyl-laurophenon

68.6 g. (0.25 moles) of 4-methyllaurophenon were poured in small portions and at a temperature of 3°-4°C into a 500 ml. beaker provided with a stirrer and a thermometer and containing 190 ml. of concentrated nitric acid. After the addition the mixture was stirred for 10 minutes and then poured into icy water cautiously. The solid precipitate was separated by filtration, washed with water, dried in the air and crystallized from methanol, thus obtaining 56.4 g. of the product. M.P. 48°-50°C.

| Analysis: | Found | Calculated |
|-----------|-------|------------|
| N%        | 4.36  | 4.39       |
| C%        | 71.16 | 71.44      |
| H%        | 9.26  | 9.15       |

#### Intermediate 23: 2-methyl-5-lauroyl-aniline

This product was obtained in the same manner as intermediate 20.

27.5 g. of the product, crystallized from ethanol, were obtained from 32 g. (0.1 moles) of intermediate 22, dissolved in 300 ml. of glacial acetic acid and 150 ml. of toluolated ethanol, and 55.8 g. of pulverized iron. M.P. 66°-68°C.

| Analysis: | Found | Calculated |
|-----------|-------|------------|
| N%        | 4.75  | 4.84       |
| C%        | 78.4  | 78.84      |
| H%        | 10.87 | 10.8       |

#### Intermediate 24: $\alpha$ -(2-chlorobenzoyl)-2-methyl-5-lauroylacetanilide

This product was obtained in the same manner as intermediate 18.

38.2 g. of a white product, crystallized from heptane, were obtained from 32.7 g. (0.116 moles) of intermediate 23 and 27.6 g. (0.122 moles) of ethyl 2-chlorobenzoylacetate. M.P. 77°-79°C.

| Analysis: | Found | Calculated |
|-----------|-------|------------|
| Cl%       | 7.63  | 7.54       |

55 Acidimetric titration from  $-\text{CH}_2$  = 98%

#### Coupler 9

This product was obtained in the same manner as coupler 1.

35.2 g. (0.075 moles) of intermediate 24 were brought to react with 10.1 g. (0.075 moles) of sulphurylchloride, thus obtaining 26.8 g. of the product. M.P. 85°-89°C.

65

Analysis: Cl% Found 10.51 Calculated 10.72  
Acidimetric titration from  $\text{CH}_2$  and  $-\text{SO}_2\text{NH}$  = 99%.

| Analysis: | Found | Calculated |
|-----------|-------|------------|
| Cl%       | 13.92 | 14.06      |

## EXAMPLE 10

Coupler 10:  $\alpha$ -(2-chlorobenzoyl)- $\alpha$ -bromo-5-[ $\alpha$ -(2-4-ditertamylphenoxy)-acetamide]-2-chloroacetanilide

29 g. (0.0485 moles) of intermediate 3 and 50 ml. of carbon tetrachloride anhydrous were mixed into a 250 ml. multi-neck flask provided with a stirrer and reflux-condenser. 8.6 g. (0.0485 moles) of N-bromo-succinimide were added thereto under stirring. The mixture was refluxed for 6 h. under stirring and the solid residue was removed by filtration. This filtrate was dried by evaporation and the residue crystallized twice from ligroin, thus obtaining 17.2 g. of a white product melting at 94°-96°C.

| Analysis: | Found | Calculated |
|-----------|-------|------------|
| Cl%       | 10.0  | 10.48      |
| Br%       | 11.88 | 11.81      |

Titration from  $\rightarrow$ CH = 98.5%.

Analysis: Titration from  $\rightarrow$ CH = 99.3%  
 $\rightarrow$ NHSO<sub>2</sub> = 99.3%.

## 5 Coupler preparation:

This coupler was prepared in the same manner as coupler 1.

61.5 g. of a white product, crystallized first from methanol and further from ethanol, were obtained from 69.3 g. (0.103 moles) of intermediate 27 dissolved in 250 ml. of dry chloroform and 14 g. (0.103 moles) of pure sulphurylchloride. M.P. 104°-105°C.

| 15 | Analysis: | Found | Calculated |
|----|-----------|-------|------------|
|    | C%        | 65.18 | 65.06      |
|    | Cl%       | 5.10  | 5.06       |
|    | H%        | 7.14  | 7.18       |
|    | N%        | 3.95  | 3.99       |

20

## EXAMPLE 11

$\alpha$ -(2-fluorobenzoyl)- $\alpha$ -chloro-5-(4-cetylbenzensulphonamide)-2-acetanilide

Intermediate 25:  $\alpha$ -(2-fluorobenzoyl)-2-methoxy-5-nitroacetanilide

This product was prepared in the same manner as intermediate 4.

162.6 g. of a straw-colored crystalline product were obtained from 137.2 g. (0.652 moles) of ethyl 2-fluorobenzoylacetate (intermediate 9) and 109.6 g. (0.652 moles) of 2-methoxy-5-nitroaniline. M.P. 153°-154°C.

|           |                                                      |
|-----------|------------------------------------------------------|
| Analysis: | Titration from $\rightarrow$ NO <sub>2</sub> = 98.9% |
|           | Titration from $\rightarrow$ CH = 99.5%.             |

Intermediate 26:  $\alpha$ -(2-fluorobenzoyl)-2-methoxy-5-aminoacetanilide

This product was prepared in the same manner as intermediate 5.

108 g. of the product, crystallized from methanol, were obtained from 160 g. of intermediate 25. M.P. 119°-121°C.

Analysis: Titration from NH<sub>2</sub> = 99.2 percent.

Intermediate 27:  $\alpha$ -(2-fluorobenzoyl)-5-(4-cetylbenzensulphonamido)-2-methoxy-acetanilide

93.2 g. (0.308 moles) of  $\alpha$ -(2-fluorobenzoyl)-2-methoxy-5-amino-acetanilide (intermediate 26), 500 ml. of anhydrous dioxane and 44.8 g. (0.37 moles) of diethylaniline were mixed into a 2 liter multi-neck flask provided with a stirrer, a reflux condenser, a thermometer and a dropping funnel. The mixture was heated up to 50°C and a solution of 123.5 g. (0.308 moles) of 4-cetylbenzensulphochloride in 150 ml. of anhydrous dioxane was dropped thereinto in one-half h. The solution, thus obtained, was stirred for 2 h. at 50°C and then poured into 3 liters of icy water under stirring and very slowly. A brown-colored product deposited and further was crystallized twice from ethanol, thus obtaining 133.6 g. of a whitish product melting at 91°-93°C.

25  $\alpha$ -(2-fluorobenzoyl)- $\alpha$ -chloro-5-[ $\alpha$ -(2-4-ditertamylphenoxy)-acetamide]-2-methoxyacetanilide

Intermediate 28:  $\alpha$ -(2-fluorobenzoyl)-5-[ $\alpha$ -(2-4-ditertamylphenoxy)-acetamide]-2-methoxyacetanilide

This product was obtained like intermediate 6.

130 g. of a white product, crystallized from ethanol, were obtained from 102 g. (0.3374 moles) of intermediate 26, from 33.3 g. of anhydrous sodium acetate dissolved in 900 ml. of glacial acetic acid and from 104.9 g. (0.3374 moles) of 2-4-ditertamyl-phenoxy-acetylchloride. M.P. 101°-103°C.

35 Analysis: Titration from  $\rightarrow$ CH = 99.8 percent. Coupler preparation:

The above-described product was chlorinated with sulphurylchloride like the previously described couplers.

40 102 g. of a white product, crystallized from ethanol, were obtained from 116 g. (0.201 moles) of intermediate 28 dissolved in 400 ml. of dry chloroform and 27.1 g. (0.201 moles) of pure sulphurylchloride. M.P. 76°-80°C.

45

| Analysis:                   | Found    | Calculated      |
|-----------------------------|----------|-----------------|
| Titration from CH = 99.32%. | Cl% 5.72 | Calculated 5.79 |

50

55  $\alpha$ -(2-fluorobenzoyl)- $\alpha$ -chloro-5-[4-dodecyl-phenyl-amino]-sulphonyl]-2-methoxy-acetanilide

Intermediate 29:  $\alpha$ -(2-fluorobenzoyl)-5-[4-dodecylphenyl-amino]-sulphonyl]-2-methoxy-acetanilide

60 28.1 g. (0.062 moles) of intermediate 20, 125 ml. of pure xylene and 1 ml. of dimethylaniline were mixed into a multi-neck flask provided with a stirrer and a Liebig condenser. The solution was brought to boil and 14 g. (0.067 moles) of ethyl 2-fluorobenzoyl-acetate (intermediate 9) were added thereto. The solution was boiled gently for 3 h. thus obtaining some 25 ml. of distillate. The solvent was removed by distillation under

## EXAMPLE 13

$\alpha$ -(2-fluorobenzoyl)- $\alpha$ -chloro-5-[4-dodecyl-phenyl-amino]-sulphonyl]-2-methoxy-acetanilide

vacuum and the residue was dissolved in ethyl ether. The solution, thus obtained, was shaken with an HCl acid solution, washed till it became neutral with water and dried on anhydrous sulphate. The oily residue was then dipped into ligroin, thus obtaining a white solid after 24 hours. M.P. 84°-86°C.

Analysis: Titration from  $-\text{CH}_2$  = 98.9%  
Titration from  $-\text{SO}_2\text{NH}$  = 99.41%.

#### Coupler preparation:

This coupler was prepared like what is described in the above-mentioned couplers.

| Analysis: | Found | Calculated |
|-----------|-------|------------|
| C%        | 66.02 | 66.84      |
| Cl%       | 5.20  | 5.50       |
| H%        | 6.72  | 6.55       |
| N%        | 4.28  | 4.34       |

#### EXAMPLE 14

##### $\alpha$ -(2-fluorobenzoyl)- $\alpha$ -chloro-[5-(2-cetoxy-phenylamino)-sulfoxyl]-2-methoxyacetanilide

###### Intermediate 30: 4-methoxy-benzensulfochloride.

This product was prepared according to the method described in J. A.C.S. 70, 375. The product melted at 42°-43°C.

###### Intermediate 31: 3-nitro-4-methoxy-benzensulfochloride.

This product was prepared according to the method described in the J. pr. Chem. [2] 74, 105. The product had a M.P. = 59°-61°C.

###### Intermediate 32: 3-nitro-4-methoxy-benzensulfo-(2-cetoxy)-anilide.

166.7 (0.5 M) of intermediate 12, 1,000 ml. of anhydrous dioxane, 89.5 g. (0.6 M) of N,N-diethylaniline were mixed into a multi-neck flask provided with a thermometer, a stirrer and reflux condenser and, when a complete solution thereof was obtained, 125.8 g. (0.5 M) of intermediate 31 added thereto. The brown-colored solution was heated at 80°±5°C for 3 h. under stirring and further diluted with 5 liters of ice water. The pH value of the suspension, thus obtained, was arranged at 3 + 4 with diluted HCl and the brown-colored solute was filtered on a Buchner filter, dried and crystallized from 2,500 ml. of ligroine, thus obtaining 240 g. of a beige product having a M.P. = 73°-74°C.

Analysis: Titration from  $-\text{NO}_2$ % = 100.73  
 $-\text{SO}_2\text{NH}$ % = 99.85

###### Intermediate 33: 3-amino-4-methoxy-benzensulfo-(2-cetoxy)-anilide.

This product was obtained from intermediate 32 according to the method described for intermediate 20. After crystallization from heptane, the product, thus obtained, had a M.P. = 72°-74°C.

Analysis: Titration from  $-\text{NH}_2$ % = 98.17  
 $-\text{SO}_2\text{NH}$ % = 100.3

###### Intermediate 34: $\alpha$ -(2-fluorobenzoyl)-[5-(2-cetoxy-phenylamino)-sulfoxyl]-2-methoxyacetanilide.

This product was obtained like intermediate 3.

38.1 g. of a white product were obtained from 41.5 g. (0.08 M) of intermediate 33, 200 ml. of xilol and 16.8 g. (0.08 M) of ethyl 2-fluorobenzoylacetate. The product was then crystallized from methyl alcohol and ligroin. M.P. = 77°-79°C.

Analysis: Titration from  $-\text{CH}_2$ % = 100.56  
 $-\text{SO}_2\text{NH}$ % = 98.26

###### 20 Preparation of the Coupler

This product was obtained like Coupler No. 1.

36.5 g. of a white product were obtained from 44.1 g. (0.0646) of intermediate 34, dissolved in 120 ml. of anhydrous chloroform and 8.72 g. (0.646 M) of pure sulfonyl chloride. The product was then crystallized from methyl alcohol and ligroin. M.P. = 68°-70°C.

Analysis: Titration from  $-\text{CH}_2$ % = 99.50  
 $-\text{SO}_2\text{NH}$ % = 101.1  
Calculated  
C% 63.62  
H% 7.02  
N% 3.90  
Cl% 4.94  
Found  
C% 63.72  
H% 7.07  
N% 3.83  
Cl% 4.95

#### EXAMPLE 15

##### $\alpha$ -(2-fluoro-4-[ $\alpha$ -(2,4-ditertamylphenoxy)-acetamido]-benzoyl)- $\alpha$ -chloro-2-methoxyacetanilide

###### Intermediate 35: ethyl 2-fluoro-4-nitrobenzoylacetate

This intermediate was prepared according to a method similar to the one followed to produce ethyl 2-chlorobenzoylacetate described in J.A.C.S. 37, 1259.

68.4 g. of a yellow oil, which was thermically unstable (at 180°C it turns black without distillation), were obtained from 90 g. (0.443 M) of 2-fluoro-4-nitrobenzoylchloride prepared according to the method described in Helv. Chim. Acta 51 (1934), 1350. Such an oil was used as it was for the preparation of the next intermediate. With a series of operations similar to those described for other couplers of the present invention, we successively obtained the following intermediates:

- $\alpha$ -(2-fluoro-4-nitro-benzoyl)-2-methoxy-acetanilide;  
- $\alpha$ -(2-fluoro-4-aminobenzoyl)-2-methoxy-acetanilide;  
and  
- $\alpha$ -(2-fluoro-4-[ $\alpha$ -(2,4-ditertamylphenoxy)-acetamide]-benzoyl)-2-methoxy-acetanilide.

The coupler of example 15 was obtained upon reaction of the last intermediate with sulfonyl chloride at room temperature with chloroform as a solvent, like that described for the hereinbefore described couplers.

The final coupler was a white powder crystallized from methanol. M.P. = 137°-139°C.

| Analysis: | Titration from<br>Calculated | -CH % = 99.14<br>Found |
|-----------|------------------------------|------------------------|
| C%        | 66.82                        | 66.94                  |
| H%        | 6.60                         | 6.66                   |
| N%        | 4.58                         | 4.51                   |
| Cl%       | 5.80                         | 5.83                   |

The couplers of the present invention may be used in conjunction with many types of silver halide emulsions suitable for color photography. They can be used for instance in silver bromide, silver chloride or silver iodide emulsions or in those emulsions containing a halide mixture, such as silver bromoiodide or silver chloro-bromide emulsions. The couplers can also be used in those emulsions which are described in U.S. Pat. Nos. 2,592,243 and 2,698,794. Such couplers can still be used in those emulsions capable of forming an image on the surface or in the interior of the silver halide grains, such as those described in U.S. Pat. No. 2,592,250.

As it is known to the man skilled in the art, the above-mentioned emulsions can be chemically sensitized either by addition of sulphur compounds, as described for instance in U.S. Pat. Nos. 1,574,944; 1,623,469 and 2,410,689; and by addition of noble metal salts, such as rhutenum, rhodium, iridium, palladium and platinum. Such emulsions can be chemically sensitized by addition of Au salts, as described in U.S. Pat. No. 2,399,083. They can be stabilized with Au salts as described in U.S. Pat. Nos. 2,597,856 and 2,587,915. The above-mentioned emulsions can be optically sensitized with apomerocyanine dyes as those described in German Pat. No. 1,009,020; in British Pat. No. 734,792; in French Pat. Nos. 1,559,295 and 2,018,196; in U.S. Pat. No. 3,574,631 and in Belgian Pat. Nos. 746,342 and 747,781.

The emulsions can contain organic stabilizers and ant-foggants of the cyclic amine type; iminoazoles, such as mercaptobenzimidazole; triazoles, such as those described in U.S. Pat. No. 2,444,608; azaindenes, such as those described in U.S. Pat. Nos. 2,444,605; 2,444,606; 2,444,609; 2,450,397; 2,723,541; 2,716,062; 2,735,769; 2,743,181; 2,756,147; 2,772,164 and E. J. Birr, Z. Wiss. Phot. 472 (1952); tetrazoles, such as 1-phenyl-5-mercapto-tetrazole; thiazoles and benzothiazoles, such as 1-methyl-benzothiazole and benzothiazole quaternary salts, as described in U.S. Pat. No. 2,131,038; mercapto-benzothiazoles, such as 1-methyl-mercapto-benzothiazole; oxazoles, thiosemicarbazides; primidines; iodonium derivatives; benzensulphyn acids; inorganic stabilizers of the zinc and cadmium salt type, such as those described in U.S. Pat. Nos. 2,839,405.

The emulsions can further contain any suitable plasticizer, known to the man skilled in the art, such as glycerin.

The emulsion may be hardened with any suitable hardener for gelatin, known to the man skilled in the art, such as aldehyde of the formaldehyde, glyoxale, succinic, glutaric and resorcylic aldehyde type; and halogen substituted aliphatic acids, such as mucochloric and mucobromic acids, as described in U.S. Pat. No. 2,080,019; or mixtures thereof, as described in U.S. Pat. No. 2,591,542.

The emulsions may have been supplied with a coating aid, known to the man skilled in the art, such as soap-nin. Any suitable base type, known to the man skilled in the art, can be used, such as cellulose triacetate, polyester, paper, polytenated paper. In the preparation of the silver halide dispersions, employed for preparing

silver halide emulsions, there may be employed as the dispersing agent for the silver halide in its preparation, gelatin or another water-permeable means of the colloidal albumin type, a cellulose derivative, or a synthetic resin of the polyvinyl type. Such material types are described in U.S. Pat. Nos. 2,286,215; 2,328,808; 2,322,085; 2,527,872; 2,541,474; 2,563,791; 2,768,154; 2,808,331; 2,852,382.

If desired a mixture of two or more of these colloids may be employed for dispersing the silver halide in its preparation.

The developing baths to be used in conjunction with the couplers of the invention are well-known to the man skilled in the art. They contain a developer of the p-phenylene diamine type, a development restrainer of the potassium bromide type, an antioxidant, such as sodium sulphite and an alkaline agent of the alkali hydrate or carbonate type. They may further contain both an antifoggant of the benzimidazole type and derivatives, of the benzothiazole type and derivatives, of the triazole and tetrazole type and derivatives, such as mercapto-derivatives; and an anticalcium substance of the alkaline phosphate and alkylendiaminopolyacetic acid type, such as for instance EDTA. Compounds known to the man skilled in the art, of the p-phenylene diamine type are those described for instance in U.S. Pat. Nos. 2,193,015; 2,656,273; 2,875,049 and in C. E. Kenneth Mees and T. H. James, *The Theory of the Photographic Process*, third edition, table 13.4, pages 264-295.

Suitable developers, which can be employed to develop photographic elements, containing the couplers of the present invention, are the sulphites, the hydrochlorides and the sulphates of:

- a. N,N-diethyl- P- phenylene diamine;
- b. N-ethyl,N- $\beta$ -methansulphonamido-ethyl-3-methyl-4-aminoaniline;
- c. N-ethyl, N-hydroxyethyl-2-methyl- p- phenylene diamine;
- d. N-ethyl, N- ydroxyethyl-p- phenylene diamine;
- e. N,N-diethyl-2-methyl-p-phenylene diamine.

#### EXAMPLE 16

6 g. of each coupler of the present invention and of the couplers A, B, C and D of the type known in the prior art were dissolved in 10 ml. of dibutylphthalate and 16 ml. of ethyl acetate and each solution was emulsified with 60 ml. of a 4 percent gelatin solution.

5 ml. of a 10 percent anionic surfactant solution were further added thereto and the emulsions, thus obtained, were diluted with 100 ml. of water. A fraction thereof containing 3 mM of a coupler was further mixed with 50 g. of a 7 percent gelatin silver chloro-bromide photographic emulsion which had not been optically sensitized.

The resulting emulsion was coated on a transparent cellulose acetate base and dried.

Two series of specimens were obtained therefrom: series A was incubated for 7 days at 22°C and 40-45 percent R.H. and series B for 7 days at 50°C and 10-15 percent R.H. Such specimens were then exposed through a grey step wedge and further developed with a developer corresponding to the following formula:

|                                            |           |
|--------------------------------------------|-----------|
| sodium-hexameta- phosphate                 | 2 g.      |
| sodium sulphite anhydrous                  | 4 g.      |
| 2-amino-5-diethylamino toluenhydrochloride | 3 g.      |
| sodium carbonate monohydrate               | 20 g      |
| potassium bromide                          | 2 g.      |
| water to make                              | 1,000 ml. |

The same specimens were then bleached and fixed and the fog and maximum optical density (Dmax) values read.

The specimens of series A were then exposed to a Xenon lamp in a fadeometer for 10 h. and the per cent decrease of optical density ( $\Delta$  %) calculated.

The following table shows both the  $\Delta$  values for each coupler examined in both specimen series A and B and the values corresponding to the fog differences ( $\Delta V$ ) between both series.

The same table also shows the maximum absorption ( $\Delta$  max), the maximum density (Dmax), and the  $\Delta$  D% (wherein D = 1.5) values referring to the specimens of series A.

Table

| Coupler | Fog A | Fog B | $\Delta V$ | $\lambda_{\text{max}}$ | Dmax | $\Delta D\%$ |
|---------|-------|-------|------------|------------------------|------|--------------|
| 1       | 0.14  | 0.19  | 0.05       | 457m                   | 2.25 | -8           |
| 2       | 0.13  | 0.16  | 0.03       | 450                    | 2.23 | -14          |
| 3       | 0.16  | 0.22  | 0.06       | 461                    | 2.23 | -11          |
| 4       | 0.18  | 0.20  | 0.02       | 450                    | 2.20 | -10          |
| 5       | 0.14  | 0.15  | 0.01       | 452                    | 2.19 | -11          |
| 6       | 0.14  | 0.17  | 0.03       | 439                    | 1.98 | -9           |
| 7       | 0.18  | 0.29  | 0.11       | 458                    | 2.1  | -6           |
| 8       | 0.20  | 0.30  | 0.10       | 458                    | 2.21 | -11          |
| 9       | 0.20  | 0.31  | 0.11       | 458                    | 1.84 | -9           |
| 10      | 0.13  | 0.13  | 0.00       | 458                    | 1.68 | -6           |
| 11      | 0.18  | 0.23  | 0.05       | 450                    | 2.12 | -4           |
| 12      | 0.17  | 0.20  | 0.03       | 448                    | 2.15 | -8           |
| 13      | 0.21  | 0.29  | 0.08       | 452                    | 1.83 | -1           |
| 14      | 0.18  | 0.30  | 0.12       | 450                    | 2.12 | -15          |
| 15      | 0.18  | 0.33  | 0.15       | 448                    | 1.80 | 0            |
| A       | 0.17  | 0.63  | 0.46       | 439                    | 2.1  | -8           |

TABLE—Continued

| Coupler | Fog A | Fog B | $\Delta V$ | $\lambda_{\text{max}}$ | Dmax | $\Delta D\%$ |
|---------|-------|-------|------------|------------------------|------|--------------|
| B       | 0.28  | 0.55  | 0.27       | 448                    | 2.15 | -31          |
| C       | 0.22  | 1.32  | 1.10       | 446                    | 2.09 | -8           |
| D       | 0.22  | 1.18  | 0.96       | 446                    | 2.2  | -10          |

I claim:

1. A silver halide photographic emulsion containing at least one two-equivalent benzoylacetanilide photographic coupler carrying on an aromatic ring thereof at least one ballasting group capable of imparting non-diffusing properties to said coupler, characterized by the fact that the coupler has a halogen atom in ortho position in the benzoyl residue, a chlorine or bromine atom as a substituent in the reactive methylene, and a hydrogen or halogen atom, or an alkyl, alkoxy, or dialkylamino group as substituent in the 2-position in the aniline residue, and a hydrogen atom or an acylamino, acyl, aryloxyacrylamino, arylaminosulfoxy or arylsulfonamido group as substituent in the 5-position in the aniline residue, the said 2-position and 5-position substituents together including alkyl groups having a total of at least 10 carbon atoms.

2. Silver halide photographic emulsions containing dispersed therein at least a coupler of claim 1 dissolved in a substantially water-imiscible organic solvent.

3. Photographic elements including a base and at least one layer of silver halide photographic emulsion of claim 1.

\* \* \* \* \*

30

35

40

45

50

55

60

65